

## UNITED STATES PATENT OFFICE

2,412,500

## FROTH FLOTATION OF SULPHIDE ORES

Arthur H. Fischer, New York, N. Y.

No Drawing. Application April 21, 1944,  
Serial No. 532,205

6 Claims. (Cl. 209—166)

1

This invention relates to the concentration of ores and has for an object the provision of certain improvements in concentration operations. More particularly, the invention contemplates the provision of certain improvements in flotation operations. A further object of the invention is to provide certain improvements in flotation methods or processes.

The invention is based on my discovery that alkyl xanthogen formates which are unsymmetrical with respect to the alkyl radicals are highly effective flotation reagents which may be employed advantageously as mineral collecting agents in conjunction with frothing agents and conditioning agents in froth flotation operations.

Alkyl xanthogen formates found most suitable for use in flotation concentration processes are those in which the larger alkyl radicals are disposed on the xanthogen side as indicated by the following structural formula:



in which R and R' are alkyl radicals and R contains the greater number of carbon atoms.

I have found that the alkyl xanthogen formates which are unsymmetrical with respect to the alkyl radicals may be employed more advantageously in various flotation circuits than those which are symmetrical. Thus, for example, a symmetrical compound comprising relatively small alkyl radicals, such as ethyl xanthogen ethyl formate, tends to break down and become ineffective in an alkaline circuit. Compounds having larger alkyl radicals substituted for or instead of one or both of the ethyl radicals have greater stability in alkaline circuits. A compound having the same larger radical substituted for or instead of the ethyl radicals on both the xanthogen side and the formate side may be of such stability as to be practically ineffective as a flotation agent. A compound having a larger radical on only the xanthogen side has desired stability without decreased floatative properties. I have found that a compound comprising on the xanthogen side an alkyl radical containing five or more carbon atoms and comprising on the formate side an alkyl radical containing a lesser number of carbon atoms generally may be employed with great advantage as a flotation agent.

2

Among the compounds found to be most effective are those comprising on the xanthogen side alkyl radicals containing five or more carbon atoms and comprising on the formate side the ethyl radical. Specific compounds which have been found to be highly effective include amyl xanthogen ethyl formate and hexyl xanthogen ethyl formate.

In practicing a method or process of the invention, a neutral, acid or alkaline circuit may be employed. The flotation reagents may be employed with particular advantage in alkaline circuits.

The flotation reagents may be employed advantageously in froth flotation operations designed for the concentration of both non-metallic minerals and metallic minerals and in froth flotation operations designed for the concentration of both oxidized ores and sulphide ores. The reagents can be employed with particular advantage in froth flotation operations designed for the concentration of copper sulphide ores and other sulphide ores.

The following examples illustrate the advantages of the reagents and processes of the invention over reagents and processes employed heretofore.

## Example I

30 Humbolt copper sulphide ore of the following composition with respect to copper was ground in water to form three separate aqueous pulps which were subjected to separate froth flotation operations in the presence of the reagents indicated with the production of concentrates and tailing products of the analyses indicated:

|                              | Test No. |      |      |
|------------------------------|----------|------|------|
|                              | 1        | 2    | 3    |
| Heads percent Cu.....        | 1.86     | 1.86 | 1.86 |
| Concentrates percent Cu..... | 14.43    | 18.1 | 17.2 |
| Tails percent Cu.....        | 1.07     | .289 | .277 |

## 45 REAGENTS, POUNDS PER TON

|                                    |     |     |     |
|------------------------------------|-----|-----|-----|
| Lime.....                          | .14 | .14 | .14 |
| Pine oil.....                      | .02 |     |     |
| Ethyl xanthogen ethyl formate..... |     | .02 |     |
| Amyl xanthogen ethyl formate.....  |     |     | .02 |
| Hexyl xanthogen ethyl formate..... |     |     |     |

## Example II

Chino copper sulphide ore of the following composition with respect to copper was ground in water to form two separate aqueous pulps which were subjected to separate froth flotation operations in the presence of the reagents indicated with the production of concentrates and tailing products of the analyses indicated:

|                                    | Test No. |       | Test No. |
|------------------------------------|----------|-------|----------|
|                                    | 1        | 2     |          |
| Heads percent Cu.....              | 1.12     | 1.12  | 10       |
| Concentrates percent Cu.....       | 15.34    | 16.48 |          |
| Tails percent Cu.....              | .68      | .18   |          |
| REAGENTS, POUNDS PER TON           |          |       |          |
| Lime.....                          | 12       | 12    | 15       |
| Pine oil.....                      | .14      | .14   |          |
| Ethyl xanthogen ethyl formate..... | .02      | .02   |          |
| Amyl xanthogen ethyl formate.....  |          | .02   | 20       |

## Example III

Utah Copper Company copper sulphide ore of the following composition with respect to copper was ground in water to form two separate aqueous pulps which were subjected to separate froth flotation operations in the presence of the reagents indicated with the production of concentrates and tailing products of the analyses indicated:

|                                    | Test No. |       | Test No. |
|------------------------------------|----------|-------|----------|
|                                    | 1        | 2     |          |
| Heads percent Cu.....              |          |       | 35       |
| Concentrates percent Cu.....       | 1.135    | 1.135 |          |
| Tails percent Cu.....              | 21.21    | 21.50 |          |
|                                    | .104     | .083  | 40       |
| REAGENTS, POUNDS PER TON           |          |       |          |
| Lime.....                          | 6        | 6     | 45       |
| Pine oil.....                      | .14      | .14   |          |
| Ethyl xanthogen ethyl formate..... | .02      | .02   |          |
| Hexyl xanthogen ethyl formate..... |          | .02   |          |

## Example IV

Copper Queen copper sulphide ore of the following composition with respect to copper was ground

in water to form three separate aqueous pulps which were subjected to separate froth flotation operations in the presence of the reagents indicated with the production of concentrates and tailing products of the analyses indicated:

|                                    | Test No. |       |       |
|------------------------------------|----------|-------|-------|
|                                    | 1        | 2     | 3     |
| Heads percent Cu.....              | 1.93     | 1.93  | 1.93  |
| Concentrates percent Cu.....       | 9.62     | 11.02 | 11.74 |
| Tails percent Cu.....              | 1.30     | .86   | .31   |
| REAGENTS, POUNDS PER TON           |          |       |       |
| Lime.....                          | 8        | 8     | 8     |
| Pine oil.....                      | .14      | .14   | .14   |
| Ethyl xanthogen ethyl formate..... | .02      | .02   |       |
| Amyl xanthogen amyl formate.....   |          | .02   |       |
| Amyl xanthogen ethyl formate.....  |          |       | .02   |

I claim:

1. The method of concentrating sulphide ore which comprises subjecting the ore in the form of a pulp to a froth flotation operation in the presence of amyl xanthogen ethyl formate.
2. The method of concentrating sulphide ore which comprises subjecting the ore in the form of a pulp to a froth flotation operation in the presence of hexyl xanthogen ethyl formate.
3. The method of concentrating copper sulphide ore which comprises subjecting the ore in the form of a pulp to a froth flotation operation in the presence of amyl xanthogen ethyl formate.
4. The method of concentrating copper sulphide ore which comprises subjecting the ore in the form of a pulp to a froth flotation operation in the presence of hexyl xanthogen ethyl formate.
5. The method of concentrating sulphide ore which comprises subjecting the ore in the form of a pulp to a froth flotation operation in the presence of a compound of the group consisting of amyl xanthogen ethyl formate and hexyl xanthogen ethyl formate.
6. The method of concentrating copper sulphide ore which comprises subjecting the ore in the form of a pulp to a froth flotation operation in the presence of a compound of the group consisting of amyl xanthogen ethyl formate and hexyl xanthogen ethyl formate.

ARTHUR H. FISCHER.